

1

2,695,250

**METHOD OF DRY CLEANING AND WEATHERPROOFING FABRICS**

William H. Shields and Joseph A. Piepmeyer, Cincinnati, Ohio, assignors to Emery Industries, Inc., Cincinnati, Ohio, a corporation of Ohio

No Drawing. Application July 28, 1951,  
Serial No. 239,188

7 Claims. (Cl. 117—92)

This invention relates to a method of dry cleaning fabrics or garments which are weather-proof or which are to be weather-proofed without impairing the water repellency thereof. This application is a continuation in part of our copending application Serial No. 111,342, filed August 19, 1949, now abandoned. In general, weatherproof or weather resistant garments, and the fabrics from which they are made, may be classified in two categories, one, the genuinely waterproof and two, the water repellent. Waterproof fabrics are those which are coated with rubber, resin, or the like, so that the coating constitutes a continuous outer surface in relation to which the fabric serves merely as backing. Rubberized fabric, oil cloth and similar products exemplify the waterproof type of fabric. In the water repellent types of fabric, no continuous coating is utilized, that is, the fabric is not of two layer construction as it is in the first type. The pores of the fabric are not filled so that it retains its primary characteristics as a fabric and the pores are susceptible to penetration by water under sufficient hydrostatic pressure.

The water repellency of the fabrics depends upon the well known hydrophobic tendency of oily and waxy materials which constitutes the essence of the lithographic process. If, for illustration, a screen were dipped in paraffin wax so that the wires were coated with a thin film of paraffin, the screen would hold water even if the pores were large enough to be readily visible to the naked eye. The threads of water repellent fabrics are impregnated with or coated by waxes such as paraffin, or water repellent resins, so that a comparable result is achieved and the fabric is waterproof for most practical purposes, although it looks like a fabric, handles like a fabric and is readily permeable to the atmosphere.

These water repellent fabrics in turn fall in two general classifications, depending upon the permanence of the water repellency. One type cannot be dry cleaned without destruction of water repellency due to the fact that the wax which imparts the water repellency to the fabric is readily soluble in dry cleaning solvent. The other type has been treated with a water repellent agent which is not removed by dry cleaned solvent and consequently can be dry cleaned without removal of the water repelling component.

There are many varieties of fabric of this general type and many of them are manufactured with materials and technique which are not matters of common or public knowledge. In general these fabrics may be compared or contrasted with the wax coated fabrics by the observation that the permanency or semi-permanency of the weatherproofing is accomplished by the physical or chemical synthesis of a water repellent compound with the textile fiber itself so that from the point of view of the dry cleaner the fiber may be regarded as an inherently water repellent fiber rather than as a water receptive fiber coated with solvent soluble wax.

Dry cleaning, however, involves the use, not only of a dry cleaning solvent, but of a dry cleaning detergent, without which the cleaning action is but partial at best. It is well recognized in the dry cleaning trade that water repellent fabrics cannot be subjected to routine dry cleaning without sacrifice of the water repellent characteristic, even if the water repellent component is not removed, or even if it is removed but replaced by subsequent treatment. Hence, in the past, it has been customary practice for dry cleaners either to wet wash water repellent fabrics,

2

or, alternatively, to subject them to partial dry cleaning in solvent devoid of detergent.

Water repellent garments are almost always outer garments and are, therefore, preferably dry cleaned rather than laundered or wet cleaned, because the water washing processes, generally, so disarrange the fabrics and loosen their nap that it is difficult or impossible to restore the garments to original shape and feel by the usual finishing operations. If the garment is cleaned in straight solvent without detergent then it simply is not thoroughly cleaned and the customer does not obtain the result which was anticipated.

The object of the present invention is to provide a method of dry cleaning water repellent fabrics with a dry cleaning solvent containing a detergent without sacrificing the inherent water repellency of the fabric. It is further our object to provide such a process which is applicable to both the water repellent type of fabric which requires replacement of wax after cleaning and the type of fabric which does not.

As stated, it has been well known through the trade that normal dry cleaning, that is, solvent plus detergent, was fatal to the water repellency of the garment, regardless of whether or not it was re-impregnated with wax after the dry cleaning treatment.

Our investigation has confirmed the heretofore unexplained deleterious action of the dry cleaning detergent and we have determined that such ill effects are due to minute traces of detergent which remain associated with the fabric, despite normal rinsing operations. In fact, these detergents are inherently such powerful surface active agents that the merest traces of them on the fabric are inimical to the water repellency which should otherwise be expected.

Dry cleaning detergents fall into two general classes; absorbefacients and soaps. Absorbefacients primarily render the cleaning solvent moisture absorbent, as disclosed in United States Patent No. 1,911,289, issued May 30, 1933, and incidentally improve the cleaning as a whole. Although the patent recites numerous examples of absorbefacients, the most effective and widely used among the absorbefacients is a product known as mahogany sulfonate, its use being more specifically disclosed in United States Patent No. 2,024,981, issued December 17, 1935.

The dry cleaning soaps usually comprise potassium oleate and mixtures of it with oleic acid and special solvents, but the various dry cleaning soaps now on the market contain a wide variety of the reaction products of alkali and alkaline earth, hydroxides, ammonium, amines and alkanolamines with the higher fatty acids, including lauric, palmitic, oleic and stearic. In general, the potassium and ammonium soaps of oleic acid are preferable for dry cleaning because of their softness and the greater ease with which they are dispersed in the dry cleaning solvent. In addition to these soaps, the dry cleaning detergents which are used as soaps, rather than as absorbefacients, may contain sulfated and sulphonated fatty oils and their salts, sulfated fatty alcohols and alkylaryl sulphonates. Many admixtures of these bodies may be used alternatively as soaps without addition of free water or as absorbefacients to facilitate the addition of free water.

In any case, these bodies are, and are used as, "surface active agents." The efficiency of the dry cleaning process as a whole is determined by the power and efficiency of these surface active agents. Therefore, the greater the efficiency of the dry cleaning process, the greater is the impairment of the water repellency of the fabric; the latter can be retained only by the sacrifice of the effectiveness of the cleaning.

We have discovered that the undesired effect of surface active agents, which may remain as traces on water repellent fabrics after dry cleaning, may be nullified by application of appropriate chemicals following the dry cleaning. These chemicals may be termed inactivators inasmuch as their presence serves to offset the presence of the surface active materials.

More specifically, we have discovered that the effects of the surface active agents may be nullified by impregnating the fabric with a metallic salt of the type of alumi-

num acetate or an alcoholate of the type of aluminum propoxide. Appropriate alcoholates have some advantages over the salts in that many of them can be dissolved directly in dry cleaning solvent whereas the salts cannot; but on the other hand, from the point of view of costs and of operating convenience in the average dry cleaning plant, it is more expedient at the present time to utilize the salts than the metal alcoholates.

Nonetheless, the use of salts poses a problem because while salts such as aluminum acetate may be soluble in water, they are not soluble in dry cleaning solvents. However, if an aqueous solution of aluminum acetate, or a like salt, is dispersed throughout the solvent, then the fabric immersed in the solvent will absorb both the water and the salt from the solvent. It is not easy to secure an appropriate dispersal or emulsion of aqueous aluminum acetate solution in solvent for the reason that most emulsifiers are in and of themselves surface active agents, and therefore tend to accentuate the deleterious effect of the traces of absorbefacient or detergent which remain after the dry cleaning. Also, an aqueous aluminum acetate solution is inherently more difficult to emulsify in dry cleaning solvent than water or most other solutions. The problem thus was to find emulsifiers for the aluminum acetate solution which would lose their surface active properties on drying and thus not offset the water repellent properties of the wax.

We have made the discovery and determination that the salts of long chain amines and volatile organic acids, such as stearic amine acetate, have the requisite properties. These compounds are effective emulsifiers for aluminum acetate solutions in dry cleaning solvents. After drying on the fabric, and particularly after the heating to which the fabric is subjected during drying and pressing, these emulsifying agents decompose and have no surface activity which impairs the water resistance of the wax with which the fibers are impregnated and coated. If desired, mechanical dispersers or homogenizers may be used in place of emulsifiers, but such practice would involve the installation of extra equipment which in most dry cleaning plants would be used only intermittently or occasionally. Further, if the dispersion is less than perfect, mottled or uneven weatherproofing is the likely consequence.

Thus, the preferred process of this invention involves the conventional dry cleaning of the garment in solvent with a surface active agent, then treatment with an aqueous dispersion or emulsion of a nullifying agent in dry cleaning solvent preferably with the assistance of a cationic type of emulsifying agent. If the dry cleaning has removed the water repellent component from the fabric it may be restored by contemporaneously, or thereafter, impregnating the garment with wax dissolved in a dry cleaning solvent.

Surprisingly, the fluid containing both nullifying and emulsifying agents has an appreciable though selective detergent effect, although not of the surface active type. Hence it has been possible in practice to substitute the materials of our invention for a portion of the normal quantity of detergents employed in dry cleaning operations. Not only are the various surface active agents nullified, but they may in some cases be partially supplanted by our process.

In practicing the process of this invention, the garments are first subjected to a dry cleaning process with a dry cleaning solvent which contains a surface active agent of the type hereinbefore described. Of these surface active agents, mahogany sulfonates are the most effective from the point of view of dry cleaning, and hence most inimicable to effective weatherproofing. Therefore, the following example of the after treatment to eliminate the surface activity is provided in relation to fabrics which have been first dry cleaned with mahogany sulfonates.

To 106.5 lbs. of molten stearyl amine, we add 18.0 lbs. of glacial acetate acid and 25.5 lbs. of commercial oleic acid. The mixture is stirred until homogeneous. This is mixed by vigorous stirring with 46.7 lbs. of water. A heavy paste results which is allowed to cool to room temperature.

We then charge a ribbon-type powder mixer with 15.0 lbs. of dry basic aluminum acetate powder, 1.8 lbs. of zinc oxide and 3.0 lbs. of the above paste and mix the two until a uniform, smooth powder, free from lumps is obtained. An emulsion is prepared from this powder by dispersing 60 grams of it in 150 ml. of dry cleaners'

naphtha and adding to this mixture with vigorous agitation 1000 ml. of hot water. This forms a heavy, white, water-in-oil type emulsion which is stable for several hours.

We then load a commercial dry cleaning washer with e. g., 46 lbs. of rainwear garments which are cleaned with an absorbefacient dry cleaners' naphtha according to established technique. The detergent solution is then removed and the washer charged with fresh solvent. Then 92 fluid ounces, or about two ounces per pound of garments, of the emulsion specified is added by pouring the emulsion slowly onto the cylinder of the washer while it is revolving. The washer is then run for 20 minutes after which garments are removed, extracted and dried. The same technique is applicable to garments which have been dry cleaned in solvents containing other absorbefacients, soaps and surface active materials.

For the purposes of this invention, the term "dry cleaning solvent" may be regarded as embracing the various petroleum solvents such as dry cleaners' naphtha, and the like, as well as synthetic solvents such as carbon tetrachloride, trichloroethylene and perchloroethylene. The nullifying agent, broadly, is a metallic compound or salt which is adapted to be decomposed by a heat such as that of the dry cleaners' pressing operation, into a water insoluble metallic compound, e. g., into a hydrated metallic oxide. Aluminum acetate is a very common example of a material of this type. For purposes of this invention, zinc, zirconium, cobalt and lead may be classed as typical of the metals which are general equivalents of aluminum. Other weak organic acids such as formic and propionic may be combined with such metals to provide water soluble salts which may be used in a fashion similar to the aluminum acetate. Suitable metallic alcoholates may also be used, such as aluminum isopropoxide, aluminum propoxide and other such alcoholates.

We have found that heating or pressing the cloth after final treatment is important to obtain a degree of water repellency suitable for customer acceptance and, within limits, the hotter the cloth is heated, the better the repellency. For example, if the cloth is treated and then dried at a temperature of 130° F. to 160° F., as is normally used in the tumbling or drying operation, the repellency will be very poor. However, if the cloth is pressed on a conventional finishing press where the temperature will probably be around 200° to 220° F., a considerable improvement in repellency will be obtained. Furthermore if the cloth is pressed on a so-called "hot head" press where the steam-heated head comes in direct contact with the cloth and the temperature may reach as high as 250° to 300° F., a still further improvement in repellency will be obtained.

In general, it is desirable to apply these nullifying compounds to the fabric in such proportions that, after drying, substantially 0.1% to 1.5% compound by weight is deposited on the fabric in dry form. If a water solution of the compound is employed, as we consider preferable, the solution should have a concentration of substantially 2½% to 7½% compound in water, by weight. The concentration in water solution should be kept within the limits specified, as too low a concentration will necessitate the absorption of a quantity of solution which may be beyond the water tolerance of the fabric being treated, while too high a concentration will entail the use of such a small quantity of solution that it is difficult to obtain even absorption of the solution by the load of fabrics. Solution in the amount of 0.5 ounce to 3.0 ounces per pound of dry clothes is preferably employed.

The type of emulsifying or dispersing agent used to disperse the aluminum acetate solution should be, first, cationic to avoid decomposition by the acidic aluminum acetate solution, second, decomposable by moderate heat to avoid adding a second wetting agent while attempting to neutralize the one already on the fabric and, third, characterized by the proper combination of hydrophilic and hydrophobic properties, or oil and water solubilities, to provide suitable emulsifying characteristics.

The compounds possessing all of these characteristics are the salts of long chain organic amines and volatile organic acids, for example the salts of formic, acetic or propionic acids and stearyl amine, distearyl amine, palmityl diethyl amine, the reaction product of one mole of stearic acid with one mole of ethylene diamine, and the amino esters obtained by condensing a fatty acid with a hydroxy amine such as triethanol amine. The

desired ratio of oil and water solubilities of the emulsifying agent, to provide the desired emulsion stability, can be achieved by the addition of modifying blending agents, oil soluble, which are compatible with the emulsifying agent, as for example stearic amine oleate.

A dispersion produced by mechanical means, such as by circulating through a mechanical pump or by injection of the water solution through an extremely fine orifice may be substituted for the emulsified dispersion.

Instead of introducing the nullifying compound in the form of an emulsion, aluminum isopropoxide may be dissolved directly in a dry cleaning solvent to provide a dilute solution, such as a 1% by weight solution, and the fabrics saturated with this solution. In such case, the amount deposited upon the fabric tends to vary with the extraction technique employed by the dry cleaner, but the general type of equipment commonly used by the dry cleaner at present provides a final deposit after drying which is satisfactory if the 1% concentration is employed.

The treatment may be applied to garments which are of the permanent water repellent type or to garments which are denuded of their hydrophobic component by the dry cleaning. It may also be applied to garments submitted for weatherproofing in addition to dry cleaning. In the latter two cases, it is necessary to impregnate the fabrics with wax, which may also be done to insure water repellency even to the permanently water repellent garments. This impregnation may be accomplished by wetting out the garments with dry cleaners' naphtha containing in solution 10% paraffin wax or an equivalent hydrophobic material such as scale wax, microcrystalline wax, japan wax, carnauba wax, vegetable waxes and various mixtures thereof. While the wax may be dissolved in the solvent to which the nullifying compound is added, we consider it preferable practice to deposit the wax by a separate dip after completion of the treatment which nullifies the surface active agent. This treatment may be applied to a load of garments to be rendered water repellent without necessarily sorting them to differentiate those which were previously treated to be permanently water repellent. On the other hand, any desired specialized water repellent material or technique of application may be utilized.

Finally the garments are dried, as by tumbling at a temperature, such as substantially 130° to 150° F., after which they are pressed by an iron or press which is heated to a temperature above 200° F. and is perhaps as much as a hundred or more degrees higher. After these finishing operations, the garments are water repellent.

Having described our invention, we claim:

1. The method of dry cleaning fabrics which are weatherproof or to be weatherproofed without impairing the water repellency thereof, said method comprising, cleaning the fabrics in a mixture of a dry cleaning solvent of the class consisting of naphtha, carbon tetrachloride, trichlorethylene and perchlorethylene and a surface active dry cleaning detergent of the class consisting of mahogany sulfonates, the soaps formed by lauric, palmitic, oleic and stearic acids with alkali and alkaline earth, hydroxides, ammonium, amines and alkanolamines, sulfated and sulphonated fatty oils and their salts, sulfated fatty alcohols and alkylaryl sulfonates, and further treating said fabric with a dry cleaning solvent of the type specified which contains a heat unstable compound which includes a metal of the group consisting of aluminum, zinc, zirconium, cobalt and lead.

2. The method of dry cleaning fabrics which are weatherproof or to be weatherproofed without impairing the water repellency thereof, said method comprising, cleaning the fabrics in a mixture of a dry cleaning solvent of the class consisting of naphtha, carbon tetrachloride, trichlorethylene and perchlorethylene and a surface active dry cleaning detergent of the class consisting of mahogany sulfonates, the soaps formed by lauric, palmitic, oleic and stearic acids with alkali and alkaline earth, hydroxides, ammonium, amines and alkanolamines, sulfated and sulphonated fatty oils and their salts, sulfated fatty alcohols and alkylaryl sulfonates, and further treating said fabric with a dry cleaning solvent of the type specified which contains a heat unstable compound which includes a metal of the group consisting of aluminum, zinc, zirconium, cobalt and lead to deposit 0.5-1.5% of said compound upon the fabrics.

3. The method of dry cleaning fabrics which are

weatherproof or to be weatherproofed without impairing the water repellency thereof, said method comprising, cleaning the fabrics in a mixture of a dry cleaning solvent of the class consisting of naphtha, carbon tetrachloride, trichlorethylene and perchlorethylene and a surface active dry cleaning detergent of the class consisting of mahogany sulfonates, the soaps formed by lauric, palmitic, oleic and stearic acids with alkali and alkaline earth, hydroxides, ammonium, amines and alkanolamines,

5 sulfated and sulphonated fatty oils and their salts, sulfated fatty alcohols and alkylaryl sulfonates, further treating said fabric with a dry cleaning solvent of the type specified which contains a heat unstable compound which includes a metal of the group consisting of aluminum, zinc, zirconium, cobalt and lead and decompressing said heat unstable metal containing compound by 10 15 20 25 30 35 40 45 50 55 60 65 70 75 80 85

depressing said fabrics at a temperature in excess of 200° F. 4. The method of dry cleaning fabrics without sacrificing the water repellency thereof, said method comprising, cleaning the fabrics in a mixture of a dry cleaning solvent of the class consisting of naphtha, carbon tetrachloride, trichlorethylene and perchlorethylene and a surface active dry cleaning detergent of the class consisting of mahogany sulfonates, the soaps formed by lauric, palmitic, oleic and stearic acids with alkali and alkaline earth, hydroxides, ammonium, amines and alkanolamines, sulfated and sulphonated fatty oils and their salts, sulfated fatty alcohols and alkylaryl sulfonates, further treating said fabric with a dry cleaning solvent of the type specified which contains a heat unstable compound which includes a metal of the group consisting of aluminum, zinc, zirconium, cobalt and lead and treating said fabrics with a weatherproofing material of the class consisting of paraffin and equivalent hydrophobic materials.

5. The method of dry cleaning fabrics without sacrificing the water repellency thereof, said method comprising, cleaning the fabrics in a mixture of a dry cleaning solvent of the class consisting of naphtha, carbon tetrachloride, trichlorethylene and perchlorethylene and a surface active dry cleaning detergent of the class consisting of mahogany sulfonates, the soaps formed by lauric, palmitic, oleic and stearic acids with alkali and alkaline earth, hydroxides, ammonium, amines and alkanolamines,

40 sulfated and sulphonated fatty oils and their salts, sulfated fatty alcohols and alkylaryl sulfonates, further treating said fabric with a dry cleaning solvent of the type specified which contains a heat unstable compound which includes a metal of the group consisting of aluminum, zinc, zirconium, cobalt and lead and treating said fabrics with a weatherproofing material of the class consisting of scale wax, microcrystalline wax, japan wax, carnauba wax, vegetable waxes, and various mixtures thereof.

55 6. The method of cleaning fabrics which are weatherproof or to be weatherproofed without impairing the water repellency thereof, said method comprising, cleaning the fabrics in a mixture of a dry cleaning solvent of the class consisting of naphtha, carbon tetrachloride, trichlorethylene and perchlorethylene and a surface active dry cleaning detergent of the class consisting of mahogany sulfonates, the soaps formed by lauric, palmitic, oleic and stearic acids with alkali and alkaline earth, hydroxides, ammonium, amines and alkanolamines, sulfated and sulphonated fatty oils and their salts, sulfated fatty alcohols and alkylaryl sulfonates, further treating said fabrics with an emulsion in dry cleaning solvent of the type specified of an aqueous solution of a heat unstable water soluble salt of a metal of the group consisting of aluminum, zinc, zirconium, cobalt and lead, in the presence of stearyl amine as an emulsifying agent, and thereafter applying heat to said fabrics in the pressing operation which is conventional in a dry cleaning process.

7. The method of cleaning fabrics which are weatherproof or to be weatherproofed without impairing the water repellency thereof, said method comprising, cleaning the fabrics in a mixture of a dry cleaning solvent of the class consisting of naphtha, carbon tetrachloride, trichlorethylene and perchlorethylene and a surface active dry cleaning detergent of the class consisting of mahogany sulfonates, the soaps formed by lauric, palmitic, oleic and stearic acids with alkali and alkaline earth, hydroxides, ammonium, amines and alkanolamines, sulfated and sulphonated fatty oils and their salts, sulfated fatty alcohols and alkylaryl sulfonates, further treating said fab-

rics with an emulsion in dry cleaning solvent of the type specified of aluminum acetate in the presence of a stearyl amine as an emulsifying agent, and thereafter applying heat to said fabrics in the pressing operation which is conventional in a dry cleaning process.

## References Cited in the file of this patent

## UNITED STATES PATENTS

| Number    | Name      | Date          |
|-----------|-----------|---------------|
| 1,990,691 | Hatfield  | Feb. 12, 1935 |
| 2,087,237 | Bolton    | July 20, 1937 |
| 2,181,691 | Bucy      | Nov. 28, 1939 |
| 2,323,387 | Edelstein | July 6, 1943  |
| 2,345,142 | Muller    | Mar. 28, 1944 |